

## UNITED STATES PATENT OFFICE

2,103,776

NOVEL GLUE PRODUCT FOR GLUING  
VENEERS AND CROSS-PLY SHEETS

Edouard Geistlich, Wolhusen, Switzerland

No Drawing. Original application December 24,  
1934, Serial No. 759,085. Divided and this ap-  
plication November 18, 1936, Serial No. 111,555  
In Germany October 28, 1933

7 Claims. (Cl. 134—23.8)

This application is a division of my application for United States patent filed December 24th, 1934, Serial No. 759,085, and has for its object a novel glue product for gluing veneers and cross-ply sheets of wood.

It is known to utilize for gluing wood solutions in water of mixtures of animal adhesives, i. e. gluten containing adhesives, such as bone, skin or leather glues, with urea, thio-urea or derivatives of the latter substances.

Glues of this kind have, however, the drawbacks of binding too slowly during applying heat to the glue joints and of being too little resistive against the influence of moisture.

It has also already been proposed to use as adhesives compositions of casein, urea, formaldehyde and water. Such adhesives are, however, not applicable for gluing wood, their usefulness being restricted to the production of surface 20 coats and plastic masses.

It is further known to render materials of glue-like nature or gelatine water soluble again by means of solutions of urea after these materials have become insoluble by effect of formaldehyde.

Thus by treating glues that had been tanned by means of formaldehyde or else gelatines with urea it is, admittedly, possible to partly recover the starting materials, for example from spent 30 roller laggings, but this regenerating operation results, due to deterioration of the agglomerated gluten molecules in such a considerable reduction of quality that the adhesive product obtained in this way is no longer applicable for gluing wood.

Furthermore, this regenerated glue lacks the 35 quality to bind under the influence of pressure and heat since for a modified regenerating operation it has been proposed to admix the urea to gluten containing substances prior to applying formaldehyde thereto with a view to affecting the applicability of the glue within wide 40 limits of temperature or in other words to provide for maintaining the adhesive product in liquid state for a relatively long time also at 45 raised temperature.

Moreover, adhesives have hitherto been used which consist of condensation products of an early stage of urea-formaldehyde, if desired in combination with a slight percentage amount (at 50 the most 10%) of glue. Adhesives of this sort, however, endure only for a limited length of time.

According to the present invention, the novel product, which can be applied for gluing veneers and cross-ply sheets of wood, is a water soluble 55 mixture of animal glue, carbamide, as for ex-

ample urea or thio-urea or derivatives thereof, and aldehydes, particularly formaldehyde or polymerides thereof such as paraformaldehyde, the relation of glue to urea varying between 3:1 to 6:1 and the relation of carbamide to aldehyde 5 between 3:1 to 2:1.

This novel product has the remarkable quality of binding under the influence of pressure and heat which hitherto was unheard of for gluten containing adhesives.

Alternatively, the animal glue can be partly replaced by filling materials, for example up to an amount of 60%.

The considerable technical advance thus obtained by means of the invention consists in the 15 novel glue product providing after its dissolution in water, at room temperature or when slightly heated (40° C.), and its application to the joining surface for a glued joint to ensue which is fast to the influence of moisture and is distinguished by the fact that even if the joining pressure is exerted at a temperature of 90° C. and more and fine veneers for example of oak or nut wood of minimum thickness are glued on, no glue 20 can penetrate through the pores of the veneer 25 to form pools on the upper side thereof.

In consequence of the high initial strength of the work blanks held together by means of the novel adhesive which strength accrues from the simultaneous presence of urea, thio-urea or derivatives of these substances, and formaldehyde, viz. polymerides or derivatives thereof, if desired in combination with filling materials, acids, acid or acid giving off salts, the glued together pieces 30 can be removed from the heated press after having been acted upon in the latter for a few 35 minutes and without being cooled off, so that considerable savings of time and heating steam are obtained. In this way is rendered possible 40 to utilize animal glues instead of casein glues 45 and artificial resin glues, which was hitherto unknown.

In distinction from the already proposed gluing methods in which foils are employed, the advantage obtained by means of the invention consists in the fact, that the temperatures and pressures required for carrying out the gluing are much lower and that the novel method is reliable even under severe conditions in which gluing by means of foils fails.

The method according to the invention permits of adapting the qualification of the adhesive to the special purpose for which it is to be used in wide limits by varying the relation of the percentage amounts of animal glue to urea, thio-

50

45

55

urea or derivates of the latter substances on the one hand and for example formaldehyde in form of its polymerides or derivates on the other hand (within the limits stated), if desired by adding indifferent finely ground or washed filling materials, as for example heavy spar. The amount of animal glue used for effecting the glue joint can be chosen up to 70% and more of the total amount of glue plus urea and formaldehyde or the equivalents thereof specified.

By addition of slight amounts of inorganic or organic acids, acid or acid giving off salts, the time required for forming a solid joint between two surfaces coated with an adhesive produced according to the invention under application of heat and mechanical pressure can be regulated.

Hereinafter two examples are given from which it will be evident in which manner the method according to the invention can be applied.

#### Example 1

10 kilograms of a mixture consisting of 78.0 percent by weight of powdered bone glue (50 meshes per square centimeter), 14.0 percent by weight of urea, 7.0 percent by weight of para-formaldehyde and 1.0 by weight of liquid paraffin are admixed to 6 to 8 liters of water of 40° C. by stirring.

The viscous solution thus obtained is for example applied to both sides of two veneers of alderwood of 1.5 millimeters thickness in thin coats, whereupon between the two alder-wood veneers an intervening ply of alder-wood of 2 millimeters thickness is inserted and on top of each alder-wood veneer a strong okoum  veneer of 1 millimeter thickness is placed.

This sheet thus composed of five plies is then subjected during 12 minutes to the action of a hydraulic heated press at a temperature of 100° C. and a pressure of 6 to 8 kilograms per square centimeter. On opening the press a five cross-ply sheet definitely glued is obtained without prior cooling.

If it is desired to produce a three cross-ply sheet 10 minutes pressing suffices under similar working conditions.

#### Example 2

10 kilograms of a mixture consisting of 27.8 percent by weight of powdered bone glue (50 meshes per square centimeter), 23.0 percent by weight of urea, 9.0 percent by weight of para-formaldehyde, 37.0 percent by weight of heavy spar or prepared chalk, 0.2 percent by weight of oxalic or lactic acid and 3.0 percent by weight of liquid paraffin are dissolved in 4 to 6 liters of water of room temperature.

The viscous solution thus obtained is for example applied to the wooden sheet carrier in a thin coat and then slightly allowed to dry, whereupon on the plating with fine veneers for exam-

ple of nut or oak-wood of 0.4 to 0.6 millimeter thickness, the assembly is inserted in the heated press. The pressing operation is effected preferably at a temperature of 90° C. and a pressure of from 3.5 to 5 kilograms per square centimeter. After 10 minutes duration the definitely veneered sheet is taken out of the press without prior cooling.

Veneers and cross-ply sheets of wood produced as specified in the above examples are devoid of any spotting by glue having penetrated to the surface and can be worked as required three hours after the pressing operation and exposed to moisture, for example to an atmosphere saturated with vapour, for weeks without danger of the individual plies of wood separating.

What I claim is:

1. A glue product comprising a water solution of an animal glue material, carbamide, and aldehydes in a relation of said glue material to carbamide varying between 3:1 and 6:1, and a relation of carbamide to aldehyde varying between 3:1 and 2:1. 20

2. A glue product comprising a water solution of an animal glue material, urea, and aldehydes in a relation of said glue material to urea varying between 3:1 and 6:1, and a relation of urea to aldehyde varying between 3:1 and 2:1. 25

3. A glue product comprising a water solution of an animal glue material, thio-urea, and aldehydes in a relation of said glue material to thio-urea varying between 3:1 and 6:1, and a relation of thio-urea to aldehyde varying between 3:1 and 2:1. 30

4. A glue product comprising a water-solution of an animal glue material, a derivate of a carbamide, and aldehyde in a relation of said glue material to said derivate varying between 3:1 and 6:1, and a relation of said derivate to aldehyde varying between 3:1 and 2:1. 35

5. A glue product comprising a water solution of an animal glue material, carbamide and formaldehyde in a relation of said glue material to carbamide varying between 3:1 and 6:1, and a relation of carbamide to formaldehyde varying between 3:1 and 2:1. 40

6. A glue product comprising a water solution of an animal glue material, carbamide, and a polymeride of formaldehyde in a relation of glue material to carbamide varying between 3:1 and 6:1, and a relation of carbamide to said polymeride varying between 3:1 and 2:1. 50

7. A glue product comprising a water solution of a mixture of animal glue material and a filling material in a proportion of the latter to the former ingredient of said mixture of about 60% by weight, carbamide and aldehydes in a relation of said mixture to carbamide to aldehyde varying between 3:1 and 2:1. 55